

## UNITED STATES PATENT OFFICE

ANTOINE MARC GAUDIN, OF BUTTE, MONTANA

## SEPARATION OF MINERALS BY FLOTATION

No Drawing.

Application filed August 19, 1930. Serial No. 476,455.

My invention relates to improvements in the separation of minerals by flotation, and more specifically relates to the treatment of ores containing sulfides in which the principal base-metal constituents are copper and zinc. One object of my invention is to provide practical means for obtaining improved yields of valuable concentrates in the treatment of ores containing both copper and zinc, and another object of my invention is to provide new and improved means for the flotation treatment of low-grade ores containing minerals separable only with great difficulty by flotation processes at present known.

There is only one common zinc-bearing sulfide known as sphalerite,  $ZnS$ . Sphalerite, however, is sometimes iron-bearing, in which case it is called marmatite,  $(Zn,Fe)S$ . On the other hand copper-bearing sulfides are numerous, and several of these are often found together in one ore. Chalcopyrite  $CuFeS_2$ , chalcocite,  $Cu_2S$ , covellite,  $CuS$ , bornite (variable, approximately  $Cu_5FeS_4$ ), tetrahedrite (approximately  $Cu_3Sb_2S_3$ ), tennantite (approximately  $Cu_8As_2S_7$ ), and enargite (approximately  $Cu_3AsS_4$ ) are the commonest. Together with minerals containing copper and zinc, copper-zinc ores frequently contain pyrite and pyrrhotite which are iron sulfide barren of copper or zinc and of the nature of undesirable impurities.

In the beneficiation of copper-zinc ores by flotation it is desired to segregate from each other (1) the copper-bearing minerals, (2) the zinc-bearing minerals, (3) the barren waste and iron sulfides, in order to smelt separately the copper-bearing and zinc-bearing products and to discard the waste.

To date the only copper-zinc ores that have been treated successfully by selective flotation are those in which the copper occurs as chalcopyrite. Successful treatment of these ores has been obtained by floating the chalcopyrite ahead of the sphalerite or marmatite, then by floating the sphalerite or marmatite ahead of the remainder of the pulp. The usual steps have been as follows:

1. The ore is ground in a circuit made slightly alkaline by the use of lime or soda ash, sometimes in the presence of a cyanide

or of zinc sulfate or of zinc oxide, or of a combination of these reagents;

2. A mineral collector such as thiocarbonilid, a xanthate or a coal-tar oil, and a froth-producer, such as pine oil or cresylic acid, are added to the pulp just ahead of, or in the flotation machines, and the copper-bearing froth is removed in the usual manner;

3. Copper sulfate and lime are added to activate the zinc mineral and inhibit the iron minerals, respectively. The pulp is conditioned by moderate agitation in a tank;

4. A mineral collector and a froth producer are added to the pulp just ahead of, or in the flotation machines and the zinc-bearing froth is removed in the usual manner;

5. Either concentrate may be cleaned by certain combinations of the above steps with or without regrinding.

I have found that this customary procedure fails when applied to ores in which the copper occurs partly or wholly in some other form than covellite or chalcopyrite. Modification of the customary procedure by substantially changing the alkalinity is of no avail as the zinc mineral floats with the copper minerals in a mixed froth. I have found, however, that a procedure which differs materially from the customary procedure and

which is actually the reverse of such procedure can be put to useful ends in some cases. Specifically, I have discovered that the zinc-bearing sulfides can be floated ahead of the copper-bearing sulfides if the copper occurs in some other form than covellite or chalcocite.

I have also discovered that if the copper-bearing material is chalcocite, a substantial modification has to be introduced in the method described above for the treatment of chalcopyritic copper-zinc ores for effective separation to result. Finally I have discovered a complex procedure which is useful in treating ores in which the copper occurs in such combination of forms as to necessitate special treatment.

I have discovered that sphalerite can be floated from a sphalerite-chalcopyrite or a sphalerite-bornite mixture and that the sphalerite of copper-zinc ores is more read-

ily floated than the chalcopyrite or bornite if the circuit is made strongly alkaline or if an oxidizing agent is added or if considerable aeration or conditioning of the 5 pulp is used, or if a combination of these effects is employed. The oxidizing agents that I have found most desirable are bleaching powder, chloride of lime, chlorine, sodium dichromate, potassium permanganate, 10 oxygen and air. Alkaline circuits made alkaline with lime have shown decided advantages over circuits made alkaline with soda as they have caused a further inhibition of the barren iron sulfides.

15 In applying my invention to ores containing copper in some other form than chalcopyrite, chalcocite or covellite, I use one of two procedures:

20 1. The zinc-bearing mineral alone is floated from the total pulp, then the copper minerals are floated from the remainder.

25 2. The copper and zinc-bearing minerals are first floated together from the total pulp. Subsequently they are separated, the zinc mineral floating and the copper minerals being inhibited.

In applying the first procedure the ore may be ground with the oxidizing agent, which may be, for example, chloride of lime 30 or chlorine gas, or after grinding the pulp may be stirred in a tank for a sufficient length of time with the oxidizing substance, for example, oxygen. Any combination of these means may also be used. In applying 35 the second procedure the combined copper and zinc minerals may be floated as usual, then separated from each other by the use of oxidizing reagents or of alkaline circuits or of a combination of these following a re- 40 grinding or a conditioning treatment or both. When using either procedure a lime circuit is desirable if barren iron sulfides are present in the ore. The inhibiting action of lime on pyrite is well-known and use of it 45 is made in a large number of plants.

In applying my invention to chalcopyrite copper-zinc ores, I prefer, first, to float as much chalcopyrite as possible away from the remainder of the pulp, as outlined above in 50 the description of the usual procedure. Secondly, I condition the copper concentrate with reagents designed to inhibit the copper, such as lime and oxidizing agents; this conditioning may be carried out in a con- 55 ditioning tank or in conjunction with a re- grinding operation. Thirdly, I float the rougher copper-concentrate so as to collect a zinc middling in the froth and a cleaned copper product in the tailing. The method 60 that I use is particularly applicable to ores in which the copper content is small com- 65 compared to the zinc content.

The following experiments indicate the character of the results that I have obtained:

65 *Example 1.*—A chalcopyrite-sphalerite-

pyrite flotation concentrate containing 17.6% copper and 6.2% zinc was aerated for fifteen minutes with potassium dichromate, 2.0 lb./ton, then for ten minutes with lime, 2.0 lb./ton. Flotation was then conducted without the use of other reagents than those already in the concentrate. The concentrate was cleaned once without the use of additional reagents. Metallurgical results were as follows:

| Product             | Weight<br>grams | Zn %  | Cu % | Recoveries % |      |
|---------------------|-----------------|-------|------|--------------|------|
|                     |                 |       |      | Zn           | Cu   |
| Rougher tailing     | 820             | 0.65  | 18.8 | 9.6          | 83.8 |
| Cleaner concentrate | 105             | 47.50 | 8.8  | 80.6         | 5.3  |
| Cleaner tailing     | 72              | 8.2   | 26.6 | 9.8          | 10.9 |

80 *Example 2.*—A synthetic mixture of 84% pure granite, 8% pure sphalerite and 8% pure bornite was ground in a pebble mill with 2.0 lb./ton lime and 2.0 lb./ton chloride of lime. A rougher zinc concentrate was obtained on addition of 0.02 lb./ton terpineol and a rougher copper concentrate on subsequent addition of 0.03 lb./ton amyl xanthate. The rougher zinc concentrate was cleaned upon addition of 0.4 lb./ton chloride of lime, and the rougher copper concentrate was cleaned after conditioning for fifteen minutes with 0.2 lb./ton chloride of lime and 0.6 lb./ton lime. Metallurgical results were as follows:

| Product                    | Copper % | Zinc % |
|----------------------------|----------|--------|
| Cleaner zinc concentrate   | 6.50     | 55.30  |
| Cleaner zinc tailing       | 5.70     | 4.40   |
| Cleaner copper concentrate | 33.80    | 32.70  |
| Cleaner copper tailing     | 49.20    | 4.50   |
| Rougher tailing            | 0.10     | 0.18   |
| Feed (calculated)          | 5.00     | 5.30   |

85 *Example 3.*—A synthetic mixture of 84% pure granite, 8% pure sphalerite and 8% pure enargite was ground in a pebble mill with 1.2 lb./ton lime and 2.0 lb./ton chloride of lime. A rougher zinc concentrate was obtained on addition of 0.04 lb./ton terpineol and 0.01 lb./ton amyl xanthate; and a rougher copper concentrate on addition of 0.06 lb./ton terpineol, 0.10 lb./ton amyl xanthate and 0.50 lb./ton sulfuric acid. Metallurgical results were as follows:

| Product                    | Copper % | Zinc % |
|----------------------------|----------|--------|
| Rougher zinc concentrate   | 5.30     | 37.20  |
| Rougher copper concentrate | 39.60    | 6.70   |
| Rougher tailing            | 0.27     | 0.20   |
| Feed (calculated)          | 3.00     | 5.30   |

90 95 100 105 110 115 120 125 130 Copper-zinc ores in which chalcocite is the copper mineral do not respond to the usual treatment given to chalcopyrite-sphalerite ores. In this instance, again, I have found that no satisfactory separation results from the use of the customary procedure. How-

ever, I have discovered some peculiarities in the action of cyanides on chalcocite which allow a modification of the customary method so as to obtain positive results.

5 It is known that cyanides inhibit the naturally activated sphalerite of many of the complex ores by dissolving the film of copper sulfide at its surface; this inhibition is permanent unless copper ions are allowed to re-  
10 activate the sphalerite. I have found that cyanides inhibit chalcocite but that this action, in contradistinction to the action of cyanides on sphalerite is not permanent, the chalcocite floating again after immersion in  
15 cyanide for a sufficient time. I believe that this is due to the consumption of cyanide by the copper mineral. I have discovered that the metals in mixtures of chalcocite and sphalerite and of copper-zinc ores in which  
20 chalcocite is the copper mineral can be segregated by selective flotation if a relatively very high quantity of cyanide is added to the pulp at a high alkalinity (over pH 10) and in the presence of a powerful collector for copper  
25 such as amyl xanthate, butyl xanthate, amyl mercaptan or benzyl mercaptan. Use of this combination of reagents results in flotation of the chalcocite but inhibition of the sphalerite. The interpretation that I place on my invention  
30 is that no flotation of either mineral takes place as long as there is a substantial concentration of free cyanide ion in the pulp, but that as soon as that concentration is reduced below a certain unknown but very small value,  
35 the collecting agent comes into play, reacting with the surface of the chalcocite or of some oxidation product thereon, thereby causing the mineral to adhere to air bubbles and report in the froth. If the pH is below 10 the  
40 cupric ion concentration seems to be sufficient to activate the sphalerite so that its rejection is unsatisfactory; if the pH is over 13, the chalcocite is difficult to collect. I prefer therefore to carry out the operation between  
45 the limits of pH 10 and 13. The quantity of cyanide added is variable, depending upon the relative quantities of the minerals and the fineness to which they have been ground. In  
50 general, however, this quantity is much larger than is generally employed for lead-zinc, copper-iron or chalcopyrite-sphalerite selective flotation operations. The quantity of cyanide should be sufficient to inhibit momentarily both the chalcocite and the sphalerite.  
55 One to four pounds is the average quantity of cyanide required per ton of mixed chalcocite-sphalerite concentrate.

In applying this invention I prefer, first, to float collectively the chalcocite with the sphalerite. To this end I use a relatively small amount of a strong collector as mentioned above. This collective concentrate I then treat with an alkali and a relatively large quantity of cyanide to substantially complete inhibition of both chal-

cocite and sphalerite. The next step is to aerate the pulp in flotation cells. This aeration results in slow flotation of the chalcocite in preference to the sphalerite. The following example illustrates the application of this invention. 70

*Example 4.*—A synthetic mixture consisting of 84% pure granite, 8% pure chalcocite and 8% pure sphalerite was ground in a pebble mill with 2.0 lb./ton soda ash, then floated with 0.04 lb./ton terpineol and 0.05 lb./ton amyl xanthate. The tailing was discarded, the concentrate cleaned once with no additional reagents then cleaned a second time with 3.0 lb./ton sodium cyanide for selection of the copper from the zinc. Metallurgical results were as follows: 75

| Product            | Copper % | Zinc % | 85 |
|--------------------|----------|--------|----|
| Copper concentrate | 67.60    | 6.70   |    |
| Zinc concentrate   | 9.20     | 56.30  |    |
| Cleaner tailing    | 2.40     | 3.00   |    |
| Rougher tailing    | 0.12     | 0.17   |    |

Copper-zinc ores in which copper occurs 90 jointly as covellite, chalcocite, chalcopyrite and as bornite, enargite, tetrahedrite or tennantite can be beneficiated by a combination of the schemes that I have just described. Preferably I proceed as follows, although 95 some modifications of this method which should be obvious from the foregoing can also be used:

1. I float the copper and zinc minerals as 100 a collective concentrate.  
2. I condition the collective concentrate with an oxidizing agent and float again. The concentrate consists essentially of chalcocite, covellite and sphalerite, and the tailing of the other copper minerals together with most 105 of the pyrite that had floated in step 1. The tailing is a finished copper product in so far as copper-zinc separation is concerned, but its grade might be raised by subsequent treatment to float the copper minerals away 110 from the impurities in it, particularly pyrite and non-sulfide gangue constituents.

3. I subject the chalcocite-covellite-sphalerite concentrate to a flotation operation after adding considerable cyanide and after bringing the pH in the range of 10 to 13. This results in flotation of the chalcocite and rejection of the sphalerite, yielding an additional copper concentrate and a zinc concentrate. 115

The following example illustrates the application of my process to an ore of the Butte district. 120

*Example 5.*—The ore consisting essentially of chalcocite, bornite, sphalerite, pyrite and 125 granitic gangue minerals was ground in a pebble mill for one hour with 0.2 lb./ton cyanide and 1.0 lb./ton lime. Flotation was accomplished by the addition of 0.02 lb./ton pine oil and 0.04 lb./ton amyl xanthate. The 130

pH of the pulp was 11.9. The rougher concentrate was conditioned for one hour with 2.5 lb./ton chloride of lime and then cleaned by flotation without additional reagents.

- 5 This yielded a sphalerite-chalcocite concentrate. The addition of 0.04 lb./ton amyli xanthate resulted in the production of a copper concentrate consisting essentially of bornite and of pyrite, and left a cleaner tailing 70 consisting essentially of gangue and pyrite. The pH of the cleaner tailing pulp was 12.1. The chalcocite-sphalerite concentrate was aerated in the flotation cell with approximately 5 pounds cyanide per ton of chalcocite-sphalerite concentrate. This segregated that product into a chalcocite recleaner 75 concentrate and a sphalerite recleaner tailing. Metallurgical results were as follows:

| 20 | Product                     | Weight<br>grams | Metal content % |       |       | Recoveries % |       |       |
|----|-----------------------------|-----------------|-----------------|-------|-------|--------------|-------|-------|
|    |                             |                 | Cu              | Zn    | Fe    | Cu           | Zn    | Fe    |
| 23 | Chalcocite con-<br>centrate | 73              | 46.30           | 24.60 | 2.80  | 22.80        | 10.50 | 0.40  |
|    | Sphalerite con-<br>centrate | 222             | 2.10            | 54.20 | 7.20  | 3.10         | 70.50 | 3.40  |
|    | Bornite concen-<br>trate    | 281             | 34.80           | 7.80  | 18.10 | 67.10        | 12.80 | 15.90 |
|    | Cleaner tailing             | 216             | 2.50            | 1.60  | 28.70 | 3.70         | 2.00  | 19.10 |
|    | Rougher tailing             | 3170            | 0.16            | 0.20  | 6.40  | 3.30         | 4.20  | 61.20 |
|    | Feed (calculated)           | 4000            | 3.70            | 4.30  | 8.10  |              |       |       |

30 Many modifications may be made without departing from the principles of my invention as herein disclosed, and accordingly no limitations should be imposed upon my invention except as indicated in the appended claims. By "chloride of lime" as used in this application is meant the commercial product so called, made by absorbing chlorine by lime, and which contains calcium hypochlorite as its active ingredient. By "oxidizing agent" as used in the claims of this application, is meant commercial bleaching powder, "chloride of lime", calcium hypochlorite, sodium hypochlorite, free chlorine, sodium dichromate, potassium permanganate, free oxygen, atmospheric air, or any oxidizing agent equivalent in action to any of the substances named. By "copper sulfide mineral" as used in the claims of this application is 40 meant any mineral comprising copper and sulfur in chemical combination, with or without the presence of iron or other element, the term "copper sulfide mineral" thus including chalcopyrite, chalcocite, covellite, bornite, tetrahedrite, tennantite, enargite, etc.

50 I claim:

1. The flotation process which comprises collectively floating chalcocite and sphalerite, 60 refloating with an agent substantially inhibiting both chalcocite and sphalerite, treating the pulp with an oxidizing agent and thereafter separating chalcocite from the pulp.

- 65 2. The flotation process which comprises

70 collectively floating chalcocite and sphalerite, refloating with sufficient cyanide to substantially inhibit both chalcocite and sphalerite, treating the pulp with an oxidizing agent and thereafter separating chalcocite 75 from the pulp.

3. The flotation process which comprises separating chalcocite and sphalerite from gangue minerals by collectively floating the chalcocite and sphalerite, treating the concentrate with sufficient cyanide to inhibit both the chalcocite and sphalerite and thereafter aerating the pulp until the inhibiting action of the cyanide upon the chalcocite is substantially reduced, and thereafter separating chalcocite from sphalerite by flotation.

4. In the separation of minerals by flotation, the process which comprises subjecting to a flotation treatment a mixture comprising chalcocite, bornite, sphalerite and pyrite in 80 an alkaline circuit, conditioning the concentrate with chloride of lime, refloating to separate a concentrate of chalcocite and sphalerite, aerating the concentrate until inhibitory factors are reduced and then floating to separate the chalcocite from sphalerite.

5. In the separation of minerals by flotation, the process which comprises subjecting a mixture comprising chalcocite, bornite, sphalerite and pyrite to a flotation treatment 90 in an alkaline circuit, separating a primary concentrate of chalcocite and sphalerite and a secondary concentrate of bornite and pyrite, and aerating the concentrate until inhibitory factors are reduced and then floating to separate the chalcocite from sphalerite.

100 In testimony whereof, I have hereunto subscribed my name this 21st day of July 1930.

ANTOINE MARC GAUDIN.

105

110

115

120

125

130